# EUROPEAN PATENT SPECIFICATION

(11) **EP 0 103 056 B1**
(45) Date of publication and mention of the grant of the patent: **17.09.1986**
(21) Application number: 82304852.5
(22) Date of filing: 14.09.1982
(51) Int. Cl.: B22F 3/24

(54) **Sintered metal body and method of making same**
Metallischer Sinterkörper und Verfahren zu seiner Herstellung
Pièce métallique frittée et son procédé de fabrication

(43) Date of publication of application: 21.03.1984
(73) Proprietor: WORCESTER CONTROLS CORPORATION, West Boylston Massachusetts 01583 (US)
(72) Inventor: Gonzalez, Ricardo, Holden Massachusetts 01520 (US)
(74) Representative: Wisher, Michael Frederick

## Description

This invention relates to sintered metal bodies, and in particular but not exclusively, to such bodies of annular configuration suitable for use as the seat of a plug valve of the ball valve kind. It is desirable to use metal seats in such ball valves under certain conditions since the resultant valve structure can resist higher temperatures and pressures than valves which use other types of seat materials such as plastics materials, for example polytetrafluoroethylene (PTFE). When a metal valve seat is employed in a ball valve, however, there is considerable friction between the ball and its seat which can cause galling problems. Therefore, in an effort to reduce such friction, it is usual for metal valve seats to be used in conjunction with trunnioned ball valve members so that the valve member is self- supporting and the friction between it and its seat is thereby limited. This, however, is a comparatively expensive construction.

Due to the above-mentioned friction problems, metallic valve seats are hardly ever used in ball type plug valves having a floating ball. United States patent 3,592,440 (McFarland) seeks to overcome some of these problems and the disclosure of this prior US patent is hereby incorporated in the present application since the US patent discloses manufacturing techniques and materials suitable for use as a first step in the method of the present invention.

The McFarland patent discloses a metal seat for use in a floating type ball valve, the seat being formed of sintered metal of which the exterior surfaces are coated with a layer of cured polymeric material which extends to some extent into the interior pores or interstices of the sintered metal body.

However, the valve seat of the McFarland patent is a porous structure which relies upon a continuous surface coating of polymeric material to provide the desired seal, or upon a caulking action of the polymeric material within the seat to effect a desired seal in the event that the polymer coating is destroyed by any means such as fire or abrasion.

We have ascertained that the valve seat of the McFarland patent being essentially porous throughout, tends to leak fluid through the seat when the seat is subjected to pressure if the integrity of the surface coating is impaired and the above-mentioned caulking effect is imperfect.

In U.S. patent 2,838,829 (Goss) there is disclosed a method of making bearings. A bearing blank produced by compression of metallic powder is sintered and then impregnated with polytetrafluoroethylene (PTFE). After such treatment, the distribution of the PTFE remains constant. The bearing blank is then coined to its final shape, leaving voids in the blank, of 3 to 5%.

An object of the present invention is to provide a method of fabricating a leak-proof seat for use in a ball valve, together with a non-porous leak-free valve seat or seal for use in a ball valve offering improvements in relation to one or more of the shortcomings of the prior art as identified above.

According to the invention there is provided a method of fabricating a leak-proof seat for use in a ball valve, together with a non-porous leak-free valve seat or seal for use in a ball valve, as defined in the accompanying claims.

In an embodiment of the present invention described below, the foregoing disadvantages of the structure disclosed in the McFarland patent are largely mitigated by providing a seat for a floating ball valve consisting of a sintered metal matrix of which the interparticulate spaces are completely filled with cured polymeric material, whereby the seat structure, in addition to being of metal construction and therefore adapted for use in those applications where metal seats are desirable, is nonporous throughout without regard to the presence or absence of a surface coating of polymeric material. While such a surface coating can be provided to achieve additional initial lubricity, the provision of such a surface coating is optional only since the cured polymeric material which fills the interstices of the sintered metal matrix and in particular the portion thereof which is adjacent the surface of the seat, provides the desired lubricity. Any increase in temperature of the seat with a resultant expansion of the polymeric material within the seat, causes an extrusion or migration of said polymeric material from the interior of the seat through the surface of the seat to provide additional lubricity. In other words, since no voids are present within the seat itself, upon expansion of the polymeric material within the seat and the resultant increase in the internal pressure of the seat, the expanded interior polymeric material is obliged to migrate through the matrix of sintered material towards the exterior surface of the seat and to exude from the matrix onto the seat surface thereby increasing the lubricity of the seat at the seat/ball interface of the valve.

A sintered metal body such as a valve member or valve seat according to the present invention can be prepared by a series of steps, and by using metal and polymeric materials in accordance with the disclosure of the above-mentioned United States patent to McFarland. A sintered metal "green compact" structure is initially fabricated in the form and shape conventionally employed for ball valve seats and members, and then the green compact is sintered to fuse adjacent metal particles to each other. Then the resultant valve member or seat is impregnated with an emulsion of uncured polymeric material having lubricity, the impregnation being effected by means of a vacuum and/or positive pressure step. The liquid vehicle employed in the emulsion is then dried, and then the residual polymeric material is cured by heating.

According to the disclosure of the above-mentioned US patent to McFarland, a valve seat prepared by a series of steps as described above is considered to be completely fabricated except for a final surface finishing step such as grinding, to provide the seat with a desired surface accuracy, and the final seat is porous throughout except for a layer of polymeric material which covers the exterior surfaces of the seat.

In contrast, in accordance with the present invention, the product of the above steps constitutes only the starting point for a further portion of the manufacturing process and, following the above-mentioned curing step, the valve seat or member is placed in a die and subjected to extremely high pressures which operate to collapse substantially all of the interparticulate cavities and voids throughout the seat onto the portions of the cured polymeric material within the sintered metal matrix. As a result, following completion of this pressure-applying step, the cured polymeric material within the sintered metal seat or member completely fills all of the collapsed interparticulate spaces within the seat and the seat is rendered nonporous throughout. The seat can then be surface-finished, if necessary, or the seat can optionally be coated with a further layer of polymeric material which is thereafter surface-finished if necessary.

Sintered metal bodies have been suggested in previous publications, see for example US patents:

In some cases the sintered metal elements are proposed to be associated with a lubricant or polymeric material, see for example the United States patents:

in addition to the above-discussed US patent 3,592,440 (McFarland). In some cases, moreover, prior workers in the field have proposed the use of a "coining" or compression of a sintered metal body-see for example the above-mentioned Chmura and Harris patents, but these proposals have been such that the resultant structure exhibits a high density or nonporous portion adjacent the surface of the body only, and a lower density porous structure underlies the surface of the body. In contrast, the pressure-applying step of the present invention is such that the valve seat or body so produced exhibits substantially uniform density throughout and is nonporous throughout.

An embodiment of the invention will now be described by way of example with reference to the accompanying drawings in which:
Fig. 1 diagrammatically illustrates a plurality of steps forming a method of making a sintered body in accordance with the present invention; and
Fig. 2 is a cross-sectional view of a valve seat manufactured in accordance with the present invention, together with an associated die utilised in the compression step of Fig. 1.

Referring to Fig. 1, in a first step 10 of the method of the present invention a quantity of powdered metal (e.g. stainless steel or bronze) is placed. in a die whose interior configuration corresponds to the configuration desired of the final structure (e.g., an annular configuration when the object being prepared is a seat for use in a ball valve), and the powdered metal is subjected to pressures of the order of 30 tons per square inch to form a unitary metal body having the desired configuration. At this point in the fabrication operation, the individual metal particles are held together simply by interparticle friction and the structure is termed a "green compact" in the parlance of the trade. In a second step 11, the green compact is then placed in a furnace and subjected to a high temperature which is less than the melting point of the metal material in the seat but which is sufficiently high to cause a coalescing of the interfaces between the various particles in the green compact to unify the structure into a sintered metal matrix. The resultant structure is porous.

In a step 12, which may be performed before, concurrently, or after steps 10 and 11, a PTFE emulsion is formed by mixing a quantity of submicron PTFE particles in an appropriate vehicle such as water, along with some wetting agents; it must be understood, however, as discussed in the afore-mentioned US patent 3,592,440 (McFarland), that other uncured polymeric materials can be employed and entrained or suspended in other liquid vehicles. The emulsion produced in step 12, and the sintered metal seat produced by step 11 are then, in a step 13, placed in a vacuum chamber, initially in spaced relation to one another, and a vacuum is applied to the chamber to remove all air from the voids or pores in the sintered metal seat. The sintered metal seat is then immersed in the emulsion, and the vacuum is broken (if desired, a positive pressure may also be introduced into the chamber) to drive the emulsion into the pores of the sintered metal seat. The resultant polymer impregnated seat is then removed from the chamber and permitted to dry, in a step 14, e.g., at a temperature which is below the boiling point of water or which is otherwise suitable to remove the water or other liquid vehicle constituents from the emulsion, leaving a residue of PTFE (and/or of whatever other polymer is employed) in the pores of the sintered metal seat.

When the liquid vehicle is removed by the aforementioned drying step, voids are created within the seat and the interparticulate spaces of the sintered metal matrix are no longer completely filled with polymer i.e., the structure at this point is still somewhat porous. Following the drying step, the impregnated seat is again placed in a furnace in a step 15, and is heated to sinter and cure the PTFE at an appropriate "Teflon-sintering" temperature, i.e. one which is considerably lower than the sintering temperature previously employed for the metal seat alone. By way of example, if the green compact prepared in step 10 constitutes stainless steel particles, it would be sintered at approximately 1371°C (2500°F) whereas Teflon is sintered (in step 15) at around 371°C (700°F). Sintering step 15 is needed to coalesce the Teflon particles, previously in the emulsion, with one another since, otherwise, the Teflon particles would be driven out of the pores in the sintered metal seat when the seat is later subjected to fluid pressure. However during this second sintering step 15, the coalescing action of the Teflon particles tends to cause some shrinkage of the PTFE in the pores of the sintered metal seat, and this, together with the voids which were created when the water or other liquid vehicle was removed or driven off in step 14, makes this structure even more porous following completion of step 15 than it was prior to the commencement of that step.

In order to render the overall structure non- porous, the structure is then subjected, in a step 16, to extremely high pressures which collapse substantially all of the interparticulate cavities and voids throughout the seat onto the enclosed PTFE or other cured polymer within the seat, to eliminate all interparticulate voids in the sintered metal seat to the extent possible, and to render the complete seat impervious to fluid flow, i.e., to make the final product "leak free" throughout. Step 16 can be effected in the manner shown in Fig. 2 wherein the annular, polymer impregnated, sintered metal seat 20, produced by method steps 1015 described above, is placed in a die 21 which has a cooperating plunger 22 that, together, define exterior surfaces which closely conform to all of the exterior surfaces of seat 20, whereafter extremely high pressures, in the order of 40 tons per square inch (6.3 tonnes per square centimetre), are applied to the seat to collapse all voids within the seat material and to render it nonporous and of substantially uniform density throughout.

The seat 20, following completion of step 16, is of sintered metal construction wherein cured PTFE (or whatever other polymer having desired lubricity is employed) fills the interparticulate spaces or collapsed voids of the sintered metal matrix throughout the body of the seat. The seat is, accordingly, nonporous throughout. Indeed, seats constructed in accordance with the present invention have been found to hold bubble tight on helium, which is a most stringent leakage test. Those incremental portions of the polymer material which are adjacent the surface of the seat act as a lubricant at said surface. Moreover, since all interparticulate voids have been collapsed by step 16, when the seat is used in an application where the temperature is higher than room temperature, the cured polymer within the seat expands but has no place to go; and the resultant expansion is therefore manifested as an increase in the internal pressure of the seat through the matrix of sintered metal material, which experiences a migration of the cured polymer toward the surface of the seat and causes some extrusion of the polymer from the seat surface to increase the lubricity of the seat at the seat/ball interface.

Following step 16, the seat may, in a step 17, be dipped in a PTFE emulsion which is much more viscous in consistency than the emulsion in steps 12 and 13, to coat the seat with a layer of Teflon® or other polymer having desired lubricity, whereafter the coating layer is again sintered and cured to provide the seat with an outer envelope which gives the seat additional initial lubricity. As indicated in Fig. 1, however, this final step is optional. Moreover, if desired, the outer polymer layer, if provided, may be characteristically coloured to clearly identify the type of seat which has been produced.

Metric equivalents of the non-metric units quoted above are as follows:

## Claims

1. A method of fabricating a leak-proof seat for use in a ball valve comprising the steps of compacting a mass of metal particles, said mass being of annular form and having a ring-shaped face adapted to be disposed adjacent to a rotary ball in a ball valve, sintering said annular mass to fuse adjacent ones of said metal particles to one another thereby to coalesce said particles into a porous metal matrix of annular form, impregnating said annular metal matrix with an emulsion consisting of uncured particles of a polymer material carried by a liquid vehicle, said impregnating step being conducted under positive pressure conditions to drive the emulsion into the interparticulate spaces in said metal matrix and to completely fill said interparticulate spaces throughout said annular metal matrix with said emulsion, drying said emulsion-impregnated annular metal matrix to remove said liquid vehicle therefrom, thereby to leave a residue of uncured polymer particles in said interparticulate spaces, and thereafter heating said annular metal matrix to sinter and cure the polymer particles which are residual in said interparticulate spaces, characterised by the step of placing said metal matrix in a die having an annular cavity whose interior shape closely conforms to the exterior annular shape of said cured polymer- impregnated annular metal matrix, and thereafter, by use of said die, applying pressure to the exterior surfaces of said annular metal matrix in a magnitude of the order of 30 to 40 tons per square inch (463 to 618 MPa) to collapse the interior of said matrix onto the cured polymer within said matrix thereby to eliminate all voids throughout the interior of said annular matrix which remain in said matrix following said drying and sinter/ curing steps, so as to render said annular matrix nonporous throughout, said pressure applying step being so conducted as to produce an annular body whose shape and dimensions are adapted for use as a ball seat in a rotary ball valve, said annular body having substantially uniform density throughout the interior of said body and at the exterior surfaces of said body upon completion of said pressure applying step.

2. A method according to claim 1 characterised by the further steps, conducted after said pressure-applying step, of coating the exterior surfaces of said annular body with a further emulsion of polymer particles, said further emulsion being more viscous than the emulsion employed in the impregnating step, and thereafter drying said coating and sintering and curing the polymer particles in said coating to enclose said annular body in an outer envelope of polymeric material.

3. A method according to claim 1 or claim 2 characterised in that said polymeric material comprises polytetrafluoroethylene.

4. A non-porous leak-free valve seat or seal comprising an annular body of sintered particulate metal forming a metal matrix which has an external shape adapted for use in a ball valve as a seat which engages a rotatable ball in such valve, and a cured polymeric material having lubricity deposited in the metal matrix, characterised in that all of the interparticulate spaces in the metal matrix comprising the interior of said annular body are completely filled with said cured polymeric material having lubricity, whereby said polymeric material renders said metal matrix nonporous throughout the interior of said body and whereby increases in the temperature of said body which result in an expansion of the polymeric material within said matrix effect an extrusion of portions of said cured polymeric material from the interior of said body to the exterior surfaces of said body which are adapted to engage the rotatable ball of a ball valve thereby to lubricate said exterior surfaces while the interparticulate spaces within the interior of said body remain completely filled with the non-extruded portions of said cured polymeric material, the exterior surface portions of said body having substantially the same density as the interior of said body.

5. A valve seat or seal according to claim 4 characterised in that said polymeric material comprises polytetrafluoroethylene.

6. A valve seat or seal according to claim 4 or claim 5 characterised in that the exterior of said seat or seal is completely covered by a layer of said cured polymeric material.

7. A valve seat or seal made by a method according to any one of claims 1 to 3.

## Patentansprüche

1. Verfahren zur Herstellung eines lecksicheren Sitzes zur Verwendung in einem Kugelventil, umfassend die Stufen des Pressens einer Masse von Metallteilchen, wobei die Masse eine ringförmige Form besitzt und eine ringförmige Fläche aufweist, die geeignet ist, in Nähe einer drehbaren Kugel in einem Kugelventil angeordnet zu werden, des Sinterns der ringförmigen Masse, um benachbarte Metallteilen aneinander zu schmelzen und diese Teilchen dabei in eine poröse Metallmatrix mit ringförmiger Form zusammenfließen zu lassen, des Imprägnierens der ringförmigen Metallmatrix mit einer Emulsion, bestehend aus nicht gehärteten Teilchen eines Polymerwerkstoffes, der von einem flüssigen Mittel getragen ist, wobei der Imprägnierschritt unter Überdruckbedingungen ausgeführt wird, um die Emulsion in zwischen den Teilchen liegenden Räume der Metallmatrix hineinzudrücken und um diese zwischen den Teilchen liegenden Räume in der gesamten, ringförmigen Metallmatrix vollständig mit dieser Emulsion zu füllen, des Trocknens der mit der Emulsion imprägnierten, ringförmigen Metallmatrix, um das flüssige Mittel von dieser zu entfernen, wobei ein Rückstand aus nicht gehärteten Polymerteilchen in den zwischen den Teilchen liegenden Räumen zurückgelassen wird, und des nachfolgenden Erhitzens der ringförmigen Metallmatrix, um die Polymerteilchen, die in den zwischen den Teilchen liegenden Räumen zurückgeblieben sind, zu sintern und zu härten, gekennzeichnet durch die Stufe des Einsetzens dieser Metallmatrix in eine Form, die einen ringförmigen Hohlraum aufweist, dessen Innenform der Außenringform der mit gehärtetem Polymer imprägnierten, ringförmigen Metallmatrix eng entspricht und dann des Anlegens von Druck auf die Außenflächen der ringförmigen Metallmatrix unter Verwendung der Form in einer Größe in der Größenordnung von 30 bis 40 t je Quadratinch (463 bis 618 MPa), um das Innere der Matrix auf das gehärte Polymer in dieser Matrix zusammenzudrücken, um so alle Hohlräume im gesamten Inneren der ringförmigen Metallmatrix zu beseitigen, die nach den Stufen des Trocknens und Sinterns/Härtens verbleiben, um so die ringförmige Matrix durchgehend porenfrei zu machen, wobei die Stufe des Druckanlegens so ausgeführt wird, um einen ringförmigen Körper herzustellen, dessen Form und Abmessungen für die Verwending als Kugelsitz in einem Drehkugelventil geeignet sind, wobei der ringförmige Körper nach Beendigung der Stufe des Druckanlegens in seinem gesamten Inneren des Körpers und an den Außenflächen des Körpers eine im wesentlichen einheitliche Dichte hat.

2. Verfahren nach Anspruch 1, gekennzeichnet durch die weiteren Schritte, die nach der Druckanlegungsstufe ausgeführt werden, des Beschichtens der Außenflächen des ringförmigen Körpers mit einer weiteren Emulsion von Polymerteilchen, wobei die weitere Emulsion viskoser ist als die in der Imprägnierstufe verwendete Emulsion und des nachfolgenden Trocknens dieser Beschichtung und Sinterns und Härtens der Polymerteilchen in der Beschichtung, um den ringförmigen Körper in eine äußere Hülle aus Polymerwerkstoff einzuschließen.

3. Verfahren nach Anspruch 1 oder 2, dadurch gekennzeichnet, daß der Polymerwerkstoff Polytetrafluoräthylen umfaßt.

4. Porenfreier, leckfreier Ventilsitz oder Dichtung, umfassen einer ringförmigen Körper aus gesintertem, teilchenförmigen Metall, das eine Metallmatrix bildet, die eine Außenform besitzt, die für die Verwendung als Sitz in einem Kugelventil, der eine drehbare Kugel in einem solchen Ventil aufnimmt, geeignet ist und einem gehärteten Polymerwerkstoff mit Schmierfähigkeit, der in der Metallmatrix abgelegt ist, dadurch gekennzeichnet, daß alle zwischen den Teilchen liegenden Räume der Metallmatrix, umfassend das Innere des ringförmigen Körpers vollständig mit einem gehärten, polymeren Werkstoff, der Schmierfähigkeit besitzt, gefüllt sind, wobei der polymere Werkstoff die Metallmatrix über das gesamte Innere des Körpers porenfrei macht und wobei Temperaturerhöhungen des Körpers, die zu einer Ausdehnung des Polymerwerkstoffes in der Matrix führen, ein Austreiben von Teilen des gehärteten Polymerwerkstoffes vom Inneren des Körpers zu den Außenflächen des Körpers bewirken, die geeignet sind, die drehbare Kugel eines Kugelventils aufzunehmen, um so die Außenflächen zu schmieren, während die zwischen den Teilchen liegenden Räume im Inneren des Körpers vollständig mit den nicht extrudierten Anteilen des gehärteten Polymerwerkstoffes gefüllt bleiben und wobei die Außenflächenteile des Körpers im wesentlichen die gleiche Dichte besitzen, wie das Innere des Körpers.

5. Ventilsitz oder Dichtung nach Anspruch 4, dadurch gekennzeichnet, daß der Polymerwerkstoff Polytetrafluoräthylen umfaßt.

6. Ventilsatz oder Dichtung nach Anspruch 4 oder Anspruch 5, dadurch gekennzeichnet, daß das Äußere des Sitzes oder der Dichtung vollständig durch eine Lage des gehärteten Polymerwerkstoffes bedeckt ist.

7. Ventilsitz oder Dichtung, hergestellt nach dem Verfahren gemäß einem der Ansprüche 1 bis 3.

## Revendications

1. Procédé de fabrication d'un siège étanche utilisable dans une vanne à boule, comprenant les opérations de compactage d'une masse de particules de métal, cette masse étant de configuration annulaire et présentant une face en forme d'anneau prévue pour être placée adjacente à une boule tournante dans une vanne à boule, de frittage de cette masse annulaire de manière à lier par fusion des particules adjacentes desdites particules de métal les unes aux autres, afin d'agglomérer ces particules en une matrice métallique poreuse de forme annulaire, d'imprégnation de cette matrice métallique annulaire avec une émulsion composée de particules non durcies d'un polymère dans un véhicule liquide, ladite opération d'imprégnation étant effectuée dans des conditions de pression positive pour repousser l'émulsion dans les espaces entre particules de la matrice métallique et pour remplir complètement avec ladite émulsion lesdits espaces entre particules dans toute la matrice métallique annulaire de séchage de cette matrice métallique annulaire imprégnée d'émulsion pour en éliminer ledit véhicule liquide, de façon à laisser un résidu de particules de polymère non durci dans les espaces entre particules, puis de chauffage de ladite matrice métallique annulaire pour fritter et durcir les particules de polymère qui restent dans les espaces entre particules, ledit procédé étant caractérisé en ce qu'il comprend la mise en place de ladite matrice métallique dans un moule comportant une cavité annulaire dont la configuration intérieure se conforme étroitement à la configuration annulaire extérieure de la matrice métallique annulaire imprégnée de polymère durci, et ensuite, au moyen dudit moule, l'appliquer d'une pression aux surfaces extérieures de la matrice métallique annulaire, d'une valeur de l'ordre de 463 à 618 MPa, de manière à écraser l'intérieur de la matrice sur le polymère durci à l'intérieur de la matrice, ce qui supprime tous les vides à l'intérieur de la matrice annulaire qui subsistaient dans la matrice après les opérations de séchage et de frittage/ durcissement, de sorte que ladite matrice annulaire devient entièrement non poreuse, l'opération d'appliçation de pression étant exécutée de manière à produire une pièce annulaire dont la forme et les dimensions sont adaptées à l'utilisation comme siège de boule dans une vanne à boule tournante, cette pièce annulaire ayant une densité sensiblement uniforme dans tout l'intérieur de ladite pièce et aux surfaces extérieures de ladite pièce après achèvement de ladite opération d'application de pression.

2. Procédé suivant la revendication 1, caractérisé en ce qu'il comprend en outre les opérations, effectuées après ladite opération d'application de pression, de revêtement des surfaces extérieures de la pièce annulaire avec une autre émulsion de particules de polymère, ladite autre émulsion étant plus visqueuse que l'émulsion employée dans l'opération d'imprégnation, et ensuite de séchage dudit revêtement et de frittage et durcissement des particules de polymère dans ledit revêtement, de manière à enfermer ladite pièce annulaire dans une enveloppe extérieure de polymère.

3. Procédé suivant la revendication 1 ou la revendication 2, caractérisé en ce que le polymère comprend du polytétrafluoroéthylène.

4. Siège, ou garniture de vanne, étanche et non poreux comprenant une pièce annulaire en particules métalliques frittées, constituant une matrice métallique qui présente une configuration extérieure adaptée à l'utilisation dans une vanne à boule comme un siège qui est en contact avec une boule tournante dans une telle vanne, et un polymère durci ayant des propriétés lubrifiantes déposé dans la matrice métallique, caractérisé en ce que tous les espaces entre particules de la matrice métallique constituant l'intérieure de la pièce annulaire sont complètement remplis avec ledit polymère durci à propriétés lubrifiantes, de sorte que ledit polymère rend ladite matrice métallique non poreuse dans tout l'intérieur de ladite pièce et de sorte que des augmentations de température de ladite pièce, qui engendrent une dilatation du polymère à l'intérieur de ladite matrice, provoquent une extrusion de portions dudit polymère durci, de l'intérieure de la pièce aux surfaces extérieures de ladite pièce qui sont prévues pour venir en contact avec la boule tournante d'une vanne à boule, afin de lubrifier lesdites surfaces extérieures tandis que les espaces entre particules à l'intérieur de ladite pièce restent complètement remplis par les portions non extrudées dudit polymère durci, les parties de surface extérieure de la pièce ayant sensiblement la même densité que l'intérieur de la pièce.

5. Siège ou garniture d'étanchéité de vanne suivant la revendication 4, caractérisé en ce que ledit polymère comprend du polytétrafluoroéthylène.

6. Siège ou garniture d'étanchéité de vanne suivant la revendication 4 ou la revendication 5, caractérisé en ce que l'extérieur dudit siège ou garniture est complètement recouvert d'une couche dudit polymère durci.

7. Siège ou garniture d'étanchéité de vanne, fabriqué par un procédé suivant l'une quelconque des revendications 1 à 3.
